

## UNITED STATES PATENT OFFICE

2,090,105

## CORROSION RESISTANT ALLOY

Carl Carius, Essen-Rellinghausen, Germany, assignor to Fried. Krupp Aktiengesellschaft, Essen-on-the-Ruhr, Germany

No Drawing. Application September 10, 1936,  
Serial No. 100,115. In Germany December 19,  
1935

2 Claims. (Cl. 75—125)

My invention relates to corrosion-resistant chromium-nickel-molybdenum-iron alloys having an addition of antimony. These alloys are remarkable for very high resistance to corrosion. 5 For example, their resistance to caustic soda solution or caustic potash solution and especially to hydrochloric acid is far superior to that of the usual chromium-nickel-molybdenum-iron alloys, for example of the known austenitic chromium-nickel-molybdenum steels. The new alloys may 10 be further improved by an addition of copper.

In my co-pending application for Letters Patent, Serial Number 28,943, filed June 28, 1935, 15 which matured into Patent No. 2,054,927 on Sept. 22, 1936, I have already suggested alloys of the following composition:

|                                                        | Percent |
|--------------------------------------------------------|---------|
| Carbon                                                 | 0.—1.   |
| Chromium                                               | 10.—25. |
| 20 Nickel                                              | 20.—40. |
| Molybdenum                                             | 1.—10.  |
| Antimony                                               | 2.—7.   |
| Copper                                                 | 0.—10.  |
| 25 Balance iron with or without the normal impurities. |         |

I have now found that the above-mentioned high resistance to corrosion of these alloys is also obtained already with antimony contents of 30 0.5 to 2%. So, for example, an alloy containing

|          | Percent |
|----------|---------|
| Carbon   | 0.04    |
| Chromium | 13.     |
| Nickel   | 30.     |

|                                        | Percent |
|----------------------------------------|---------|
| Molybdenum                             | 5.      |
| Copper                                 | 5.      |
| Antimony                               | 1.5     |
| Balance iron with the usual impurities | 5       |

has been tested in 25% hydrochloric acid solution at a temperature of 80° centigrade. The loss in weight occurring by this treatment amounted only to from 1 to 2 grammes per sq. meter per hour. 10

Preferably I use alloys of the following composition:

|                                                     | Percent  |
|-----------------------------------------------------|----------|
| Carbon                                              | 0.02—0.2 |
| Chromium                                            | 10. —20. |
| Nickel                                              | 27. —33. |
| Molybdenum                                          | 2. —5.   |
| Copper                                              | 2. —6.   |
| Antimony                                            | 0.5 — 2. |
| Balance iron with or without the normal impurities. | 20       |

What I claim and desire to secure by Letters Patent is:—

1. A chromium-nickel-iron alloy containing 25 0.02—1% carbon, 10.—25% chromium, 20.—40% nickel, 1.—10% molybdenum, 0.5 to less than 2% antimony, 0.1—10% copper, balance iron with or without the normal impurities.

2. A chromium-nickel-iron alloy containing 30 0.02—0.2% carbon, 10.—20% chromium, 27.—33% nickel, 2.—5% molybdenum, 2.—6% copper, 0.5 to less than 2% antimony, balance iron with or without the normal impurities.

CARL CARIUS.